

1

2,750,732

**SELF-IGNITING FUEL AND A METHOD OF  
USING SAME**

Paul C. Condit and Manuel A. Pino, Berkeley, Calif., assignors to California Research Corporation, San Francisco, Calif., a corporation of Delaware

No Drawing. Application October 29, 1951,  
Serial No. 253,749

7 Claims. (Cl. 60—35.4)

This invention relates to propellant fuel compositions which are characterized by self-ignition when mixed with powerful oxidizing agents and to particular mixtures of these fuels and oxidizing agents.

Self-igniting compositions of various kinds have for many years found use in the construction of assorted tools of war for use against personnel and property. More recently, it has been recognized that self-igniting compositions are useful as propellants for rockets, guided missiles, and aircraft powered by jet or thrust engines.

In the development of fuels for rockets, thrust engines, etc., it has been recognized that the property of self-ignition in the propellant fuel, while not absolutely essential, constitutes a major convenience in the construction and operation of these devices. In the development of rocket fuels, two types have been recognized: monergols, or monergols, i. e., unitary compositions which require ignition by spark, pyrotechnic charge or otherwise and, once started, they continue to burn on being sprayed into the hot zone; and hypergolic fuels, or hypergols, which comprise two or more components which are separately stored and which spontaneously ignite upon proper mixing in a combustion chamber. The individual components of the hypergolic mixture are not self-igniting.

Monergols so far developed have proved unreliable in that they have all shown a tendency to backfire from the combustion chamber to storage tanks. This difficulty is not encountered with hypergolic fuels since self-ignition occurs only upon mixing of the individual components which are not themselves self-igniting and neither of which alone has the property of undergoing self-sustained combustion after ignition.

Hypergolic propellants may be generally described as mixtures of a reducing component and an oxidizing component. When the two components are mixed, there is a short period during which the mixture exists as a composition of matter. During this short period relatively slow reaction of the two components is apparently initiated and this relatively slow reaction is followed by spontaneous ignition of the fuel. The ignition delay period is quite short, being substantially less than one second and being preferably not more than about fifty milliseconds.

The reducing component of a hypergolic propellant should have certain properties as follows: It should ignite spontaneously upon being combined with the selected oxidizing agent; the ignition delay period should be short, preferably not exceeding 50 milliseconds; it should have a low freezing point so that it can be pumped to the combustion chamber at the low temperatures prevailing at high altitudes; it should have a high boiling point to facilitate handling and increase its safety in use; it should be chemically stable in storage; it should have a relatively low viscosity at low temperatures; it should form gaseous oxidation products and the average molecular weight of these products should be as low as possible in order that the specific impulse (pounds thrust/pounds propellant/

2

second) be high. In addition to the foregoing properties, it is desirable that self-ignition of the mixture of the reducing component and the oxidizing agent be rapid over a wide temperature range; that the reducing component have a high density so that the volume of fuel tanks may be reduced; that the material be non-toxic and easy to handle; that it have a high heat of combustion; and that it be non-corrosive.

It has now been found that the foregoing property requirements are satisfied in a remarkable degree by a self-igniting propellant composition consisting essentially of at least one material of the group consisting of acyclic mercaptans containing from 1 to 5 carbon atoms, especially primary and secondary mercaptans, and an oxidizing agent consisting predominantly of fuming nitric acid.

It has further been found that mercaptans produced by separating mercaptans from thermally cracked naphtha and fractionally distilling the separated mercaptans to recover a fraction boiling within the range from 125° F. to 300° F. constitute a highly satisfactory reducing component for a hypergolic propellant. This mercaptan fraction is characterized in that it is self-igniting when mixed with concentrated nitric acid.

The reducing component of the above-described hypergolic propellant may be methyl mercaptan, ethyl mercaptan, normal propyl mercaptan, isopropyl mercaptan, normal butyl mercaptan, isobutyl mercaptan, secondary butyl mercaptan, allyl mercaptan, normal amyl mercaptan, secondary amyl mercaptan, unsaturated C<sub>3</sub>—C<sub>5</sub> mercaptans, or a mixture of two or more of these materials. Tertiary butyl mercaptan and tertiary amyl mercaptans are satisfactory if mixed with at least 50% by volume of one or more of the primary and secondary mercaptans named.

The oxidizing component of the above-described hypergolic propellant is predominantly fuming nitric acid, that is, nitric acid having a purity in the range from 95% to 100% HNO<sub>3</sub> by weight. Commercial fuming nitric acid composed of 98.5% by weight of HNO<sub>3</sub> and 1.5% by weight of water is satisfactory. A small amount of N<sub>2</sub>O<sub>5</sub> may desirably be added to commercial fuming nitric acid to render it anhydrous.

It has been found that the ignition delay period observed when fuming nitric acid is mixed with the mercaptans above described may be considerably shortened by incorporation in the nitric acid of a minor proportion of a material which functions as an ignition accelerato. One such material is nitrogen dioxide which may be added in amounts from 2% to 20% by weight, ordinarily about 7½% by weight being employed. The nitrogen dioxide imparts a characteristic reddish color to the acid and this mixture is sometimes referred to as red fuming nitric acid. A second material which may be added to fuming nitric acid to accelerate ignition is sulfuric acid. This material is also added in amounts from 2% to 20% by weight, from 12% to 15% by weight being ordinarily employed. A third material which may be added to fuming nitric acid as an ignition accelerator is nitrosyl sulfuric acid. This material is also employed in amounts from 2% to 20% by weight, about 15% being desirably employed.

The following examples illustrate the propellant of this invention:

**EXAMPLE 1**

One volume of ethyl mercaptan and three volumes of fuming nitric acid containing 15% by weight of sulfuric acid were mixed at —40° F. Ten milliseconds after mixing, spontaneous ignition of the mixture occurred. The mercaptan was very rapidly oxidized forming water vapor, carbon monoxide, carbon dioxide and sulfur dioxide and the acid was reduced forming water vapor, nitrogen and nitrogen oxides. The ignition delay is measured by mixing



ing 15% by weight of sulfuric acid as the oxidizing agent. Runs were made at sea level at temperatures of 75° F., -12° F. and -31° F. In all cases the engine started and operated satisfactorily. Runs were made at a pressure altitude of about 50,000 ft. at temperatures from -27° F. to -73° F. Satisfactory starts in performance were obtained in all runs. Eleven successful runs at 50,000 ft. at a temperature of approximately -70° F. clearly demonstrated the reliability of the starting characteristics of this propellant combination. The engine was very clean after repeated runs using the mixed mercaptans and the above-described acid.

A number of performance tests were made in a 220 pound thrust rocket engine to determine the effect of varying the acid mercapton ratio in the combustion chamber of the engine. Using the mercapton mixture described in Example 9 and white fuming nitric acid, a ratio of acid to mercaptans of 4.2:1 would be stoichiometric for complete oxidation of the mercaptans. It was found that the specific impulse, i. e., the number of pounds thrust per pound of fuel per second, went through a maximum as the ratio of acid to mercapton was varied and that this maximum existed when the acid content of the acid mercapton mixture was from about 80% to 95% of stoichiometric. Further tests with pure mercaptans showed that similar maxima existed for mixtures of these materials with fuming nitric acid and with fuming nitric acid containing the ignition promoters described herein. Accordingly, it is preferred to operate thrust engines using acid and mercapton injection rates such that the acid mercapton ratio is 5% to 20% below stoichiometric.

The foregoing examples have been limited to illustrations of self-igniting mixtures of the mercaptans alone with fuming nitric acid. It is not necessary, however, that pure mercaptans be used. In practical operation it is possible and often desirable to blend the mercaptans with up to 50% by volume of hydrocarbon fuel.

#### EXAMPLE 17

Individual mercaptans and the mixed mercaptans of Example 9 were diluted with a straight run petroleum distillate and red fuming nitric acid was added to the resultant mixture at room temperature. The maximum amounts of distillate which could be added to the mercaptans without losing the property of self-ignition upon addition of nitric acid were determined. The distillate employed in the tests tabulated below had a 10% point of 215° F. and a 90% point of 250° F. on an ASTM D-86 distillation and contained 43% paraffins, 48% naphthenes, and 9% aromatics. Approximately equivalent results were obtained with cracked distillates and with wider boiling cuts such as gasoline and kerosene.

| Mercapton           | Maximum Dilution with Petroleum Distillate for Self-Ignition with Fuming Nitric Acid |
|---------------------|--------------------------------------------------------------------------------------|
|                     | Vol. percent                                                                         |
| Isopropyl mercapton | 30                                                                                   |
| n-propyl mercapton  | 30                                                                                   |
| t-butyl mercapton   | 30                                                                                   |
| n-butyl mercapton   | 20                                                                                   |
| Mixed mercaptans    | 30                                                                                   |
| Allyl mercapton     | 60                                                                                   |

The ignition accelerators described above were effective with the mercapton-hydrocarbon oil-nitric acid mixtures in about the same manner as with mercapton-nitric acid mixtures.

#### EXAMPLE 18

Although it has been found that pure tertiary mercaptans are not self-igniting in  $HNO_3$ , considerable concentration of the  $C_4$  or  $C_5$  tertiary compounds may be present

in the primary or secondary mercaptans of this invention without seriously restricting the utility of these materials as propellents. The exact quantity of tertiary mercapton that can be tolerated will depend upon the intended use, but it may be as high as 30 to 50%. In some cases it may be more practical to manufacture such mixtures than it is to make the pure primary and secondary mercaptans, and mixtures of primary and/or secondary mercaptans containing substantial quantities of tertiary mercaptans are, therefore, within the scope of this invention.

The self-igniting character of mixtures of tertiary mercaptans with non-tertiary mercaptans is evidenced by the following tabulated results obtained pursuant to the method of Example 1, using a mixture of sulfuric and white fuming nitric acids as the oxidizing agent.

|    | Vol. percent Sec.-butyl Mercapton | Vol. percent t-butyl Mercapton | Temp., °F. | Ignition Delay, Milli-seconds |
|----|-----------------------------------|--------------------------------|------------|-------------------------------|
| 20 | 25                                | 75                             | 75         | 14                            |
|    | 75                                | 25                             | -40        | 12                            |
|    | 50                                | 50                             | -40        | 12                            |
| 25 | 90                                | 10                             | -70        | 30                            |
|    | 75                                | 25                             | -70        | 30                            |
|    | 50                                | 50                             | -70        | 31                            |

The mixtures of primary and secondary mercaptans with the tertiary mercaptans should contain at least 50% by volume of the primary and secondary mercaptans and preferably should predominate in these materials if overall satisfactory properties, including freezing point, are to be insured.

Obviously, many modifications and variations of the invention as hereinbefore set forth may be made without departing from the spirit and scope thereof, and only such limitations should be imposed as are indicated in the appended claims.

40 We claim:

1. The method of starting a fire by autoignition which comprises mixing at least one mercapton of the group consisting of primary and secondary acyclic mercaptans containing from 1 to 5 carbon atoms per molecule with an oxidizing agent consisting predominantly of fuming nitric acid.

2. A fuel, characterized in that it is self-igniting upon addition of concentrated nitric acid, consisting essentially of a mixture of acyclic mercaptans containing 1 to 5 carbon atoms per molecule, said mixture containing at least 50% by volume of mercaptans selected from the group consisting of primary mercaptans and secondary mercaptans.

3. The method of operating a thrust engine which comprises introducing a mixture of acyclic mercaptans containing from 1 to 5 carbon atoms per molecule, said mixture containing at least 50% by volume of mercaptans selected from the group consisting of primary mercaptans and secondary mercaptans, and fuming nitric acid into the combustion chamber of the engine to form an ignited propulsion charge and ejecting the burning charge from the combustion chamber at high velocity.

4. The method as defined in claim 3, wherein the quantity of fuming nitric acid introduced into the combustion chamber is from 80 to 95% of the amount stoichiometrically required to oxidize the mercaptans.

5. The method as defined in claim 1, wherein the nitric acid contains a minor amount in the range from about 2 to 20% by weight of sulfuric acid.

6. The method as defined in claim 1, wherein the nitric acid contains a minor amount in the range from about 2 to 20% by weight of nitrosyl sulfuric acid.

7. The method as defined in claim 1, wherein the nitric

acid contains a minor amount in the range from about 2% to 20% by weight of nitrogen dioxide.

References Cited in the file of this patent

UNITED STATES PATENTS

1,742,263 Koch ----- Jan. 7, 1930

|             |                       |               |
|-------------|-----------------------|---------------|
| 2,033,877   | Burk -----            | Mar. 10, 1936 |
| 2,328,709   | Crandall et al. ----- | Sept. 7, 1943 |
| 2,489,051   | Sayward et al. -----  | Nov. 22, 1949 |
| 2,557,018   | Viles -----           | June 12, 1951 |
| 5 2,573,471 | Malina et al. -----   | Oct. 30, 1951 |